

## UNITED STATES PATENT OFFICE

2,166,338

## DEEP-DRAWING ZINC ALLOY

Kurt Bayer, Magdeburg, and Arthur Burkhardt, Berlin-Lichterfelde, West, Germany, assigns to Georg von Giesche's Erben, Breslau, Germany, a corporation of Germany

No Drawing. Application October 25, 1937, Serial No. 170,854. In Germany December 4, 1936

2 Claims. (Cl. 75—178)

Our invention relates to copper-zinc alloys, and more particularly to alloys for the production of deep-drawing sheets.

It is an object of our invention to provide an alloy of the kind referred to which is more suitable for deep drawing than the alloy known as "63 brass", i. e., brass containing 63 per cent copper, employed almost exclusively for deep drawing heretofore.

10 To this end, we provide an alloy containing 4 to 5.5 per cent copper, 0.1 to 0.2 per cent aluminium, and zinc which is practically free from magnesium and cadmium as the remainder.

Heretofore, there has been no lack of endeavours to replace the usual 63 brass by low-copper zinc alloys, and particular advantages were expected from the use of pure zinc.

Thus, it was attempted to roll into deep-drawing sheets the usual zinc die-casting alloys, with 20 their high elongation, but the attempt failed as such alloys can be rolled into sheets only with difficulty or not at all, the sheets which could be obtained possess, if any, only very limited deep-drawing capacity, and even this decreases with ageing.

25 We have made the surprising discovery that these difficulties are overcome by determining the composition of the alloy as stated above, i. e., 4 to 5.5 per cent copper and 0.1 to 0.2 per cent aluminium, and omitting the addition of magnesium made in the said die-casting alloys for suppressing intercrystalline corrosion, and cadmium, by using zinc practically free from these admixtures.

30 Investigations have demonstrated that even an addition of magnesium of only 0.002 per cent in a copper-aluminium-zinc alloy reduces its deep-drawing capacity to half, and an addition of 0.01 per cent magnesium reduces it to  $\frac{1}{4}$  of that in an alloy without magnesium.

35 The influence of cadmium is also detrimental, an addition of 0.002 per cent reducing the deep-drawing capacity by about 10 per cent, and an addition of 0.01 per cent reducing it by about 25 per cent.

40 The following table shows the influence of magnesium and cadmium on the deep-drawing capacity.

| 50 | Composition of alloy, per cent |     |       |       |           | Erichsen deep-drawing values for sheet 0.4 millimeter |
|----|--------------------------------|-----|-------|-------|-----------|-------------------------------------------------------|
|    | Cu                             | Al  | Mg    | Cd    | Remainder |                                                       |
| 55 | 5                              | 0.2 |       |       | Zinc      | 19                                                    |
|    | 5                              | 0.2 | 0.002 |       | do        | 11                                                    |
|    | 5                              | 0.2 | 0.01  |       | do        | 5.5                                                   |
|    | 5                              | 0.2 | 0.02  |       | do        | 5.5                                                   |
|    | 5                              | 0.2 |       | 0.002 | do        | 17                                                    |
|    | 5                              | 0.2 |       | 0.01  | do        | 14                                                    |
| 60 | 5                              | 0.2 |       | 0.05  | do        | 13                                                    |

It appears that even a very small admixture of magnesium must be avoided, the more so as the alloys must be resistant to ageing, and that cadmium is also undesirable.

Omission of aluminium would not result in any appreciable advantage with respect to ageing resistance while on the other hand it would involve the drawback that the alloys could not be melted in iron containers, as iron is strongly attacked by zinc alloys without aluminium.

By extensive investigations we have found that an alloy containing 4 to 5.5 per cent copper, not more than 0.2 per cent aluminium, and zinc practically free from magnesium and cadmium as the remainder, is absolutely resistant to ageing.

The indicated content of aluminium so far reduces the dissolving capacity of the alloy for iron that the alloy can be melted in iron containers without difficulty. On the other hand, 0.2 per cent is the upper limit since alloys containing more aluminium are not resistant to ageing.

The composition of our alloy may be varied, as shown by the following examples:

|        | Per cent Cu | Percent Al | Remainder                             | 25 |
|--------|-------------|------------|---------------------------------------|----|
| 1..... | 4           | 0.1        |                                       |    |
| 2..... | 5           | 0.1        |                                       |    |
| 3..... | 5           | 0.2        |                                       |    |
| 4..... | 5.5         | 0.1        |                                       |    |
| 5..... | 5.5         | 0.2        | Zinc practically free from Mg and Cd. |    |
|        |             |            |                                       | 30 |

Sheets rolled from such alloys have a tensile strength of 28 to 33 kilogrammes per square millimeter, and an elongation of 60 to 40 per cent, as against rolled 63 brass, with a tensile strength of 29 to 35 kilogrammes per square millimeter, and an elongation of about 45 per cent.

35 Sheets from the new alloys according to our invention are preferably rolled crosswise, and preferably at temperatures ranging from 180 to 220 centigrade.

40 The following table shows the result of a comparative test between sheet rolled from the alloy (2) of the table of compositions, and 0.4 millimeter thick, and sheet of 63 brass of equal thickness. The test was made by the Erichsen method in conformity with the Werkstoff-Handbuch for non-ferrous metals, sheet B7.

| 50 | Alloy                                             | Tensile strength, kg/mm <sup>2</sup> | Elongation, per cent | Erichsen deep-drawing values    |
|----|---------------------------------------------------|--------------------------------------|----------------------|---------------------------------|
|    | 5 percent Cu, 0.2 percent Al, remainder zinc..... | 28 to 33<br>29 to 35                 | 60 to 40<br>45       | Millimeters<br>18 to 19<br>12.2 |
|    | 63 brass.....                                     |                                      |                      | 55                              |

45 The Erichsen value of alloy (2) is 18 to 19 mm., as against 12.2 mm. in 63 brass.

50 The following table shows the Erichsen values

of various alloys as a function of their copper content.

| 5  | Composition of alloy, percent |     |      | Erichsen deep-drawing values for sheet 0.4 mm. thick |
|----|-------------------------------|-----|------|------------------------------------------------------|
|    | Cu                            | Al  | Zn   |                                                      |
| 10 | 6                             | 0.2 | 93.8 | Millimeters                                          |
|    | 5                             | 0.2 | 94.8 | 18 to 19                                             |
|    | 4                             | 0.2 | 95.8 | 16                                                   |
|    | 3                             | 0.2 | 96.8 | 12                                                   |
|    | 2                             | 0.2 | 97.8 | 9                                                    |
|    | 1                             | 0.2 | 98.8 | 8                                                    |

15 The best Erichsen values were obtained with the alloys having 6 and 5 per cent copper, 0.2 per cent aluminium, and electrolytic zinc of high purity and free from magnesium and cadmium, as the remainder.

20 By way of comparison, it may be mentioned

that the Erichsen value of electrolytic zinc having a purity of 99.99 per cent, and a tensile strength of 20 kg./qmm., is 11 mm.

As mentioned, sheets from our alloys are preferably rolled crosswise, and at 180 to 220 centigrade. Temperatures above and below this range are detrimental to the deep-drawing capacity of the sheet.

We claim:

1. An alloy containing from 4 to 5.5 per cent 10 of copper, from a small but effective amount up to 0.2 per cent of aluminium, the remainder being zinc practically free from magnesium and cadmium.

2. An alloy containing from 4 to 5.5 per cent 15 of copper, 0.1 to 0.2 per cent of aluminium, the remainder being zinc practically free from magnesium and cadmium.

KURT BAYER.

ARTHUR BURKHARDT. 20